

Sept. 11, 1962

L. K. SCHUSTER ET AL

3,053,702

METAL COATING

Filed May 19, 1959.

Fig. 2.



Fig. 1.



INVENTORS

222

Ludwig K. Schuster  
Alfonso L. Baldi, Jr.

BY Connolly and Hutz

ATTORNEYS

## 1

3,053,702

## METAL COATING

Ludwig K. Schuster, Philadelphia, and Alfonso L. Baldi, Jr., Drexel Hill, Pa., assignors to Pennsalt Chemicals Corporation, Philadelphia, Pa., a corporation of Delaware

Filed May 19, 1959, Ser. No. 814,200  
16 Claims. (Cl. 148—6.2)

The present invention relates to the coating of metal, particularly for reducing the corrosion of the metal and for giving it a colored appearance, and represents an improvement in the subject matter of U.S. Patents 2,768,103, 2,768,104, both granted October 23, 1956, and 2,773,623 granted December 11, 1956. This application is in part a continuation of applications Serial No. 587,388, filed May 25, 1956 (now U.S. Patent 2,911,332, granted November 3, 1959), Serial No. 666,852, filed June 20, 1957, Serial No. 708,772, filed January 14, 1958 (now abandoned but replaced by Serial No. 88,018, filed February 9, 1961), and Serial No. 738,648, filed May 29, 1958.

Among the objects of the present invention is the provision of coating compositions and methods, as well as coated products, that are relatively inexpensive yet give very good results in both protecting against corrosion and imparting a pleasing appearance.

The above as well as additional objects of the present invention will be more clearly understood from the following description of several of its exemplifications, reference being made to the accompanying drawings wherein:

FIG. 1 is a partially broken away view of a can coated in accordance with the present invention; and

FIG. 2 illustrates a baling strap coated in accordance with the present invention, the strap being shown in place around a bale, part of the coating being removed so as to better show it.

Although the application of chromium oxide coatings reduced in situ from aqueous solutions of chromic acid and compatible reducing agents, as described in the above-listed U.S. Patents 2,768,103, 2,768,104 and 2,773,623, provide very good protection against corrosion, the coatings so produced are not very decorative. By suitable adjustment of the coating solution formulations, the coatings can be made brown in color but the brown is very frequently mottled by interference fringes that spoil its appearance, apparently by reason of its fairly transparent nature.

According to the present invention pigments can be incorporated in the above type of coatings to make them present very attractive appearance, but special provision is required to make the pigments compatible. Also unless the non-pigment ingredients are adjusted in proportion so as to avoid the prior brown colorations, the effect of all but the darkest pigments is largely lost. In other words, the prior brown colorations, although sufficiently transparent to be beset by interference fringes, are still capable of seriously masking the effect of pigments, even those that impart brown colors.

In order to bring out the above advantageous coloring, the chromic acid is replaced by the water soluble dichromate of a metal having a valence greater than one. To avoid the brown coloration the proportion of reducing agent is adjusted so that at least 70% of the hexavalent chromium is reduced to trivalent condition in the final coating. Accordingly, of the 40 to 95% range of reduction disclosed in the above patents, only the uppermost portion is used.

Suitable pigments for the purpose of the present invention are the more inert ones such as titanium dioxide, carbon, iron oxide and the phthalocyanine pigments such

## 2

as phthalocyanine blue and phthalocyanine green. Also effective is finely divided metallic zinc which, though having relatively low tintorial ability, greatly increases the corrosion protection which the coatings provide. The pigments give their best hiding when in very finely divided form, as for example when the pigment particles are about one micron or smaller in size, but the increased protection by the zinc powder reaches a maximum when the powder particles are about 50 microns in size. In general, pigment is preferably dispersed in the coating solution in a proportion of from 10 to 75% by weight of the dichromate content. Wetting agents, particularly of the non-ionic type, are advantageously used to keep the pigment particles dispersed during the coating process.

To give a more brilliant appearance and good corrosion resistance the coatings should also have a minimum coating weight of at least about 100 milligrams per square foot of surface covered. Resins are also best included in the coating, as set forth in the above-identified parent applications, inasmuch as such additions further improve the corrosion protection and also make it easier to apply very heavy coatings. Coating weights as high as 1000 to 2000 milligrams or more per square foot can be readily applied in this way. Too much resin renders the final coating sensitive to the action of solvents which can cause the color to become streaky as well as dulled. To avoid this the maximum resin content should be no higher than 1 part by weight for every 3 parts of dichromate content by weight in the coating dispersion. Excellent protection is obtained, however, with resin to dichromate ratios as high as 2 and as low as 0. The best overall results are in the resin to dichromate range from 1.5:1 to 1:3. Wetting agents also preferably of the non-ionic type are helpful in keeping the resin particles dispersed in the coating mixture. The above ratios are calculated by comparing the resin weight to the difference between the weight of the metal dichromate and the weight of the cation of the dichromate.

A feature of the present invention is that even without resin the presence of pigments improves the corrosion resistance contributed by the coating. Phthalocyanine blue and  $TiO_2$  are particularly effective in this respect.

Acrylic resins such as methyl acrylate, ethyl acrylate and methyl methacrylate resins are a preferred type of resin. They can be provided in hardnesses of Tukon 2 or more, and where the coated product is to be subjected to handling, softer resins, particularly in amounts larger than 1 part by weight for every 2 parts by weight of dichromate in the coating dispersion, cause the final coating to become more or less readily marked by finger prints and the like. Hard pigments like  $TiO_2$  also reduce the susceptibility to marking.

The pigment-containing coatings of the present invention are applicable to any material that can withstand the application conditions. Even paper can be so coated. However, the invention is of primary significance in connection with the coating of metals by reason of the high corrosion resistance which the coating contributes. Indeed, the corrosion resistance is of such magnitude that the coating will even protect such metals as chromium-nickel stainless steels (18-8 for instance) which are relatively slow to corrode. The coating also adheres very well to corrodible metals although in some case, as with aluminum and stainless steels, it may be helpful somewhat to roughen the surface of the metal slightly, or else not to polish the surface too much when the metal is manufactured. Roughening can be effected by etching or abrasion, as with sand blasting, or even by rolling the metal between rough surface rollers. In the case of plain carbon steels and iron, roughening is not needed to improve the adhesion of the coating, but the corrosion protection of such metals can be sharply increased by giving

them a preliminary grain boundary etch, as described in applicants' prior application Serial No. 592,552, filed June 20, 1956, now Patent No. 3,031,333. The coatings of the present invention can also be applied very effectively over metals that have been given a prior adherent coating of oxide or other materials such as phosphate, oxalate, sulfide or other chromate coatings, including those used to improve the adhesion of paint to ferrous metals as well as to lubricate those metals for working operations. Examples of such preliminary treatments are given in the above-identified U.S. Patent 2,768,104.

Coatings of the present invention when so applied over the pre-coated metals give much better protection against corrosion as compared to pre-coated metals when they are not given a second coating. It is also noted that a water-base paint when applied over such double coated metals, also gives much better corrosion resistance, and for this purpose the coating of the present invention need not have any resin or pigment present and can even be applied in very thin films. Thus, a 20 milligram per square foot coating from an aqueous solution of only zinc dichromate and a compatible reducing agent like sucrose, so as to cause 70 to 95% reduction of the hexavalent chromium to trivalent form when this solution is subjected to the curing step, makes a very desirable covering over plain carbon steel that has been phosphatized, as shown in Examples 13 and 14 of the above-identified Patent 2,768,104. The zinc-dichromate-reducing-agent solution can be merely applied in the form of a final rinse after the phosphatizing operation, particularly when the material being treated is a formed object such as an automobile frame or chassis. A similar improvement is obtained with such formed objects that are first given a grain boundary etch, then coated with the zinc-dichromate-reducing agent mixture, and after curing, given a final coat of water-based paint. Similar results are also obtained with such formed objects when  $\text{CrO}_3$  is used in place of zinc dichromate in each of the above modifications.

Metals suitable for treatment in accordance with the present invention, in addition to the stainless steels, plain carbon steels and aluminum mentioned above, include straight chromium steel, beryllium, cadmium chromium, cobalt, columbium, copper, lead manganese, magnesium, molybdenum, nickel, silver, tantalum, tin, titanium, vanadium, zinc, zirconium, and alloys of any of these metals with each other.

For avoiding color appearance on very bright surfaces such as stainless steel and aluminum, polytetrafluoroethylene can be used in a mixture that leaves a coating weight of 1.5 milligrams per square foot. For such treatment there can be used a coating mixture of

6 grams zinc dichromate  
2 grams sucrose  
4 cc. of an aqueous dispersion of polytetrafluoroethylene having 50% resin solids content by weight  
0.05 gram p-octyl phenyl tri-oxyethylene ethanol diluted to 4 liters with water.

A dip in the above formulation followed by heating of the dipped product at 400° F. to cure the coating left by the dip, provides a 3 milligram per square foot protective layer that imparts very good corrosion resistance to stainless steel articles such as automobile windshield wiper arms. Most of the cured coating is in powdery form and will readily rub off on handling, without detracting from the corrosion resistance but improving the appearance by rendering the protective coating invisible. In the above formulation the resin-to-dichromate ratio can be varied over the 1.5:1 to 1:3 range mentioned earlier, and in fact the resin can be entirely omitted although this diminishes the corrosion protection somewhat. The resin-free coating does not powder off but can be buffed off as described in patent application Serial No. 666,852. Also the zinc dichromate of the above formulation can be replaced by strontium dichromate, or calcium dichromate or even

$\text{CrO}_3$  with not much loss of effectiveness. The curing can take place at any temperature between 250° and 450° F.

The following example gives one typical technique for providing the pigmented coatings of the present invention:

#### Example I

An aqueous dispersion is prepared with the following formulation:

64 cc. of an aqueous solution of zinc dichromate containing 0.75 gram per cc. of chromium as  $\text{CrO}_3$ .  
32 cc. of an aqueous solution of sucrose containing 1/2 gram of sucrose per cc.  
60 cc. of an aqueous dispersion of three parts of carbon black to one part of phthalocyanine blue, the dispersion containing 1/10 gram of solids per cc. and stabilized with 0.1% addition by weight of hydroxy ethyl cellulose.  
30 cc. of an aqueous polymethyl methacrylate resin dispersion containing 13 grams of polymer having an average molecular weight of 10,000 and a Tukon hardness of 4, stabilized with 0.1% of the ammonium salt of 4-isopropyl naphthalene sulfonic acid.

The above ingredients are diluted to 600 cc. with water and SAE 1010 steel strapping is dipped in it following which the strapping is rolled between grooved rollers. The resulting wet metal is passed through an air oven where it momentarily reaches a temperature of 350° F. The resulting article has a coating that weighs 200 milligrams per square foot and has a very pleasing black appearance. It also withstands a 98% humidity test at 95° F. for 100 hours without showing a sign of attack. The coating adheres very well, cannot be scraped off with the finger nail, and does not take any impression by pressing a finger against it.

Similar results are obtained over the entire range of coating formulations as set out above, except that other resins such as polystyrenes and the butadiene-styrene copolymers described in parent application Ser. No. 708,772, filed January 14, 1958, will take a mark corresponding to a finger print if they have a Tukon hardness of less than about 2. The coatings that are free of resin or contain not more than one part of marking resin for every three parts of dichromate in the coating dispersion, do not show marking.

The above coatings also produce a very pleasing leather-like appearance when applied over metal that has been roughened by rolling with rough rollers, and type 302 stainless steel panels roughened in this way and coated as per Example I, give an unusually attractive appearance. Although as indicated above curing temperatures of 250 to 450° F. can be used with pigment-free coatings, the higher conversion needed for pigment-containing coatings requires a minimum curing temperature of about 280° F.

Although  $\text{TiO}_2$  is a white pigment, it normally colors the coating a pastel green, and when combined with phthalocyanine blue it will provide a darker green color. When mixed with carbon black it gives a pleasing grey. Phthalocyanine green also supplies a green color, red iron oxide a red color, and phthalocyanine blue a striking blue color.

The coating solution can also be applied by spraying, and by adjusting the spray operation, the aqueous medium of the coating dispersion can be caused to evaporate in considerable proportions before the spray particles reach the surface being coated. Thus the addition of air jets surrounding the spray jet can be arranged to evaporate as much as 3/4 of the water in the traveling of the sprayed particles to the surface being coated. As a result, the sprayed particles deposit on the surface in a more or less viscous form which does not run to any appreciable degree and furthermore builds up quite readily to give coatings weighing as much as 5,000 milligrams per square foot. This type of coating is of special significance in the treatment of fabricated articles where running of the

coating is to be avoided. Regardless of the coating thickness, the curing operation can be completed in a few seconds.

Where a large proportion of non-marking resin such as the above acrylate resins are desired and the metal after coating is to be worked as by a deformation operation, it is helpful to plasticize the resins as with polyvinyl stearate or other plasticizing agents such as acrylate resins having molecular weights of about 2000. The polyvinyl stearate can be one produced by reacting polyvinyl alcohol with sufficient stearoyl chloride to cause about half of the hydroxyl content of the polyvinyl alcohol to become esterified, or can be a fully esterified material such as made in the manner described in U.S. Patents 2,188,864 and 2,562,965. The plasticizer can be added in an amount up to about 25% of the weight of any plasticized resin and the metal so coated is suitable for high speed stamping operations such as in the making of tops and bottoms for cans used in conventional canning.

FIG. 1 shows such a can 10. The can has a tubular body 12 made in the conventional manner from a single strip of a full bright finished black plate 10 mils thick with the ends joined together as indicated at 13. These ends are folded back on each other to provide interlocking flanges 16 and 18 between which a yielding gasket layer 17 such as rubber is applied. The flange and gasket combination is then crimped together to make a suitably sturdy and leak-proof joint.

The openings at the top and bottom of the tubular body are sealed with covers 20, 22 that have beaded peripheries 24 with interlocking flanges 26, 28. Circular strengthening ribs 36 can also be formed in the top and bottom. The interlocking beaded periphery can merely be crimped, preferably with a layer 30 of gasketing to assure hermetic sealing.

As shown by the broken-away edge 32, the metal of the can body as well as the top and bottom, has a coating 34 applied in accordance with the present invention. This coating was provided on the unfabricated sheet by subjecting it to the following operations:

#### Example II

A. Clean the black plate cathodically in an aqueous solution containing 16 grams KOH per liter using a current density of 15 amperes per square foot of cathode at 140-160° F. for 10 seconds.

B. Cold water rinse.

C. Clean anodically in an aqueous solution containing 16 grams KOH per liter using a current density of 15 amperes per square foot of anode at 140-160° F. for 10 seconds.

D. Cold water rinse.

E. Flood with a passivity-preventing 1/2% by weight aqueous H<sub>2</sub>SO<sub>4</sub> solution for 1/2 second at 80° F.

F. Cold water rinse.

G. Spray with an aqueous solution containing 2% nitric acid at 80° F. for 8 seconds, using a spray pressure of about 6 pounds per square inch.

H. Cold water rinse.

I. Desmut by brushing in water to remove loose or non-adherent reaction products including any developed in step G.

J. Flood for 2 seconds with a 75° F. aqueous solution of:

840 cc. of a 46% solids dispersion of a thermosetting butadiene-styrene resin similar to that described in Example 1 of U.S. Patent 2,683,698 but using styrene in place of the mixed vinyl toluenes, and omitting the sodium bicarbonate;

12 grams p-octyl phenyl tri-ethylene oxyethanol;

112 grams sucrose;

375 grams of a 36% TiO<sub>2</sub> dispersion in water;

600 cc. of an aqueous zinc dichromate solution containing

3/4 gram dichromate measured as CrO<sub>3</sub>, per cc;

600 grams zinc dust; all diluted to 6000 cc.

K. Roll through rubber rolls wetted with the flooded solution.

L. Cure by passing the resulting filmed metal through a drying unit having a set of ceramic gas burners heated red hot by burning gas, a five second exposure to the incandescent units being used, and the metal reaching a temperature of 350° to 400° F.

If the metal is in the form of an elongated strip, it may be coiled up directly after step L. The resulting coating weighs approximately 200 milligrams per square foot.

The same coated sheet, which in the above example is colored pale green, can be used for making both the top and bottom 20, 22 of the can as well as the body 12 (FIG. 1) by stamping and crimping operation, although in some cases different thicknesses of metal can be used in the different portions of the can so that separate coated sheets are required.

After the can body is secured together in the above manner, or by soldering, the cover on one end may be applied in any convenient manner such as the one generally used in the industry and shown in FIG. 1. The can can then be filled and the remaining cover applied with the usual precautions where the contents have to be sterilized or heated or kept in a special atmosphere such as under evacuation or superatmospheric pressures. The corrosion resistance of the thus treated metal is outstanding and is better than that of tin-plated cans. The cans having the coating of the present invention are particularly useful in storing such materials as detergents, soaps and other alkaline compositions, and are also suitable for holding chemicals and other items that are neutral or acid in reaction.

The stamping of the can tops, as shown in FIG. 1, involves a fairly abrupt deformation of the margin 38 to provide a backing for the bead crimping operation. The presence of the pigment does not significantly detract from the effectiveness of the coating in withstanding such deformation. However, when resins are used in an amount less than one part by weight for every one part of dichromate by weight, the resin is preferably of the butadiene-styrene type or contains about 10 to 25% plasticizer.

Another very effective treatment is with softer acrylate resins, as follows:

#### Example III

The procedure of Example II is followed except that step J is carried out by rolling the metal between rough rubber rolls wet with the following dispersion:

48 grams CrO<sub>3</sub> reacted with ZnO to form zinc dichromate; 16 grams sucrose;

60 cc. of 26% by weight aqueous dispersion of phthalocyanine blue;

37 grams of methyl acrylate resin having a Tukon hardness of 1.2 and in the form of a 46% dispersion in water; all diluted to 500 cc.

In addition, the curing temperature is reduced to about 320° F. A very attractive and protective deep blue finish results.

Inasmuch as cans generally carry lithographed or paper labels which may completely cover the body 12 and only leave the top and bottom exposed, the coloring of the present invention can be limited to only the top and bottom. The remainder of the can may be made from

metal coated in other manners such as with the pigment-free coatings of patents numbered 2,768,103, 2,768,104 and 2,773,623 as well as application Serial No. 738,648. The omission of the pigment means that thinner coatings can be used, particularly if of the resin-free type. The

coatings on the inside and outside surfaces of the can body and/or can ends, need not be the same. The outer surfaces can, for example, be of the pigmented type containing zinc either as pigment or as a sublayer (see Example IV), while the inner surfaces can have the pigment-free and zinc-free coatings. The fact that

good protection can be obtained even with extremely thin coatings such as those weighing about 20 milligrams per square foot, makes such coatings also valuable for the treatment of such materials as filters or the like, and even for such articles as television picture tube masks or screens.

For color television picture tubes, masks that provide the three-color separation for individual elements of the screen can be made by etching or otherwise forming fine apertures in a sheet of metal such as iron or copper, and the completed mask can be coated with a dilute aqueous solution of 2% chromic acid and 3/4% reducing agent such as triethanolamine, after which the mask can be drained to free it from excess solution and then heated to 250° F. to cure the coating. Substitution of zinc dichromate for all or part of the chromic acid is to be avoided in such uses inasmuch as such substitution makes it more difficult to adequately outgas the tube. The chromic acid type coatings, even though they appear to be hydrated, do not complicate the outgassing treatment which the inside of the tubes must undergo.

An exceptionally effective coating according to the present invention uses a thin undercoat of electrodeposited zinc. A typical technique of this type is:

#### Example IV

SAE 1020 steel sheet is cleaned in a 2% aqueous NaOH dip at 180° F., rinsed with cold tap water and then electrolyzed as a cathode in the following bath:

60 grams per liter of Zn(CN)<sub>2</sub>;  
23 grams per liter of NaCN; and  
53 grams per liter of NaOH.

The current density is adjusted to 11 amperes per square foot of cathode, the bath temperature to 45° C., and the electrolyzing continued until a 150 milligram per square foot layer of zinc is deposited. The zinc-covered metal is again rinsed with tap water, and sprayed with the following aqueous formulation:

|                                              | Percent |
|----------------------------------------------|---------|
| Zinc dichromate                              | 45      |
| Sucrose                                      | 8.1     |
| Thermosetting butadiene-styrene resin solids | 27.2    |
| Polyvinyl stearate                           | 9.4     |
| TiO <sub>2</sub>                             | 9.5     |
| p-Octyl phenyl tri-ethylene oxyethanol       | 0.8     |

The sprayed metal is cured at 375° F. to leave a coating weighing 200 milligrams per squared foot. The resulting coated product withstands corrosion better than aluminum-painted steel, even in sharply deformed areas.

Other pigmented coatings of the present invention are formed from formulations such as

#### Example V

To 6000 cc. water are added

4 grams of p-octyl phenyl tri-ethylene oxyethanol  
500 grams SrCr<sub>2</sub>O<sub>7</sub>  
300 grams phthalocyanine green, and  
140 grams citric acid.

This produces dark green coatings weighing about 250 milligrams per square foot and having very good corrosion resistance on steel, aluminum, cooper and brass, when cured at 375° F.

#### Example VI

1000 cc. water  
100 grams MgCr<sub>2</sub>O<sub>7</sub> made by reacting 7 parts of MgCO<sub>3</sub> with an excess (11 parts) of CrO<sub>3</sub>  
40 grams H<sub>3</sub>PO<sub>3</sub>  
30 grams red iron oxide  
4 grams dioctyl sodium sulfosuccinate.

This produces a resin-free red coating having very good protective qualities for steels, when cured by flaming so that the steel reaches a maximum temperature of 325° F.

Flaming can also be very efficiently used to cure the resin-containing coatings of the present invention, and in fact is suitable for drying or curing any kind of organic coat such as water-based paints, water-dispersed resin, and even paints having organic thinners. Where the thinners are combustible most of the thinner should be evaporated off before the paint layer reaches the flaming zone.

The coating dispersions of the present invention can tolerate a small amount of excess CrO<sub>3</sub> as indicated by the formulation of Example VI. Resin can also be present along with the excess CrO<sub>3</sub> as for instance by adding to the formulation of Example VI 50 grams of the alkyd resin of Example I in U.S. Patent 2,634,245 emulsified with 1/4 the amount of polyethylene glycols there described.

FIG. 2 shows an application of the present invention where the coloring is more significant than the corrosion resistance. A bale 40 of cotton, for example, is here shown as held by baling straps 41, 42 coated in accordance with the present invention. These straps can be of standard types of steels such as ordinary SAE 1010 or SAE 1020 steel, preferably given an extra severe rolling operation to increase the springiness and hardness of the steel somewhat. Before or after the steel is slit into the final width, generally 1/2 to 3/4 inch, it is conveniently coated in the manner set out above in Example I using a pre-etch, giving a product that is very desirable and inexpensive to manufacture. The grain boundary etch sharply increases the corrosion resistance and is valuable where straps are exposed to severe corrosion conditions. Although that etch can be omitted (along with the preliminary passivity prevention treatment), the industry does expect to have baling straps colored in the manner that they have been for the past fifty years or more, and it is this color which the present invention provides in a simple, inexpensive and attractive fashion.

The grain boundary etch as with nitric acid in the manner shown in Example II or in U.S. Patent application Serial No. 592,552, filed June 20, 1956, is also helpful for use with electrodeposited coatings. Tin plated on black plate that has been pre-etched in this manner to remove 300 milligrams of metal per square foot, shows much better corrosion resistance whether or not the tin plating is covered with the reduced chromic acid or reduced dichromate coating. Unprotected tin plated from acid electroplating baths is particularly improved by this pre-etching when in plating thickness of from 1/4 to 1 or more pounds per base box, although alkaline deposited tin plate is also improved. Grain boundary etches that remove from about 50 to about 400 milligrams per square foot are very effective in providing this improvement.

The dichromate coating solution or dispersion can be applied by immersion, flooding, spraying, roller coating, electrostatic spraying, etc. Roller coating, immersing and flooding are particularly suitable for continuous coating of strip metal. The thickness of the coating depends upon the concentration of the mixture, and if applied by roller coating, the roll pressure and roll surface characteristics also affect the thickness of the final coating.

A further feature of the present invention is that the pigment-containing coating dispersions generally do not need any supplemental wetting agent addition to help wet metals being treated. It appears that the pigment-carrying dispersions with sufficient stability to hold the pigment suitably dispersed have very good wetting characteristics regardless of the metal being coated. This is even more marked where the dispersions have resin as well as pigment stably dispersed. The use of dispersions is also associated with a drop in the criticality of the pre-cleaning step.

The dispersing or wetting agents used to stabilize the dispersions can be of any kind. In addition to those named above, long-chained alkyl sulfates are suitable and tertiary butyl alcohol will be effective although it does not cause any appreciable chemical reduction and is generally required to be in higher concentration, e.g. 0.5%,

to provide really effective wetting. In general, however, anionic, cationic or non-ionic wetting agents including quaternary ammonium compounds of long-chain alkyl or aralkylamines, can be used.

The coatings of the present invention can also be applied to glass for the purpose of reducing its attack by etching agents such as hydrofluoric acid. This feature is a great help in the manufacture of television picture tubes with glass envelopes, where the tubes have external metallic supports that are anchored to the glass envelope by means of a fritted glass block or disc fused to the envelope and providing an internally enlarged socket within which a headed-over metal arm is held. By applying the coating of the present invention to the glass frit and if desired to the adjacent portions of the metal arm, the tube envelope can be subjected to the ordinary processing involved in the conventional manufacture without having the frit attacked to the point where its anchorage to the glass envelope is dangerously weakened. Both resin-free and resin-containing coatings can be used for this purpose, and in addition, the dichromate can be replaced by chromic acid either completely or partially. Pigments need not be used in such protective coatings although they are helpful.

Another feature of the coatings of the present invention is that they can be used to reduce the corrosion of plain carbon steel razor blades of the type used in shaving, for example. In this connection coatings which may or may not have resin are preferably applied in relatively thin layers directly over the cutting edge of the razor. A coating weight of only about 30 milligrams per square foot is adequate for this purpose, and such coatings are helpful in reducing somewhat the initial keeness of the edge. As a result, the tendency for a shaver to cut his face with a brand new blade is greatly diminished. However, the corrosion protection preserves the cutting edge between shaves so that it can be used for at least as many shaves as unprotected edges.

As indicated above, the coatings of the present invention are also applicable as top coatings to sharply increase the protection of metal given a preliminary coat with other types of protective material. Such preliminary coatings can be of the phosphatizing type or of the oxide type, or of the standard coloring preparations such as those used for coloring zinc black.

In addition, because of the purely inorganic nature of the resin-free coatings of the present invention, the coatings can be applied to protect articles that have a temperature too high for other types of protection. Instances of such use are metal castings which can begin to oxidize after they are removed from the casting mold and during the time they cool down to room temperature. Aluminum or zinc castings can accordingly be sprayed with the coating dispersions of the present invention when their temperatures are as high as 500° F. or even higher. These high temperatures cause the coating to be promptly cured, and when the temperature is very high can begin to decompose the coating. However, even as so decomposed, oxidation of the metal is sufficiently inhibited during the cooling process as well as for days thereafter. A small amount of resin can even be present in such coatings and no pigment need be used. For such protection of pigs used to replenish molten metal baths, it is also preferred to apply only a very thin coating using simple solutions of chromic acid and polyalcohol reducing agent such as sugar. Less foreign material is introduced into the bath in this way, although not much is added by replacing the CrO<sub>3</sub> with one of the dichromates.

Throughout all the above ranges of formulation, the proportion of ingredients is always adjusted so that at least 40% and not more than 95% of the hexavalent chromium becomes converted to trivalent chromium when the curing is completed. However, as pointed out above, the pigment-containing mixtures should stay within the range of 70% to 95% conversion. A pigment like

TiO<sub>2</sub> is particularly desirable in that it increases the ductility of the coating so that it better protects metal that is subsequently drawn or pressed. Accordingly, when a green or blue color is desired, the colored pigment is advisedly used in combination with a liberal amount of TiO<sub>2</sub>. In Example II, for instance, the substitution of 100 parts of phthalocyanine green for an equal amount of the TiO<sub>2</sub> gives a good green color on a product that is more fully protected in areas that are to be deformed. The presence of the TiO<sub>2</sub> also gives the coating better hiding qualities and as pointed out above, makes the coating harder than TiO<sub>2</sub>-free pigments do.

Obviously many modifications and variations of the present invention are possible in the light of the above teachings. It is, therefore, to be understood that within the scope of the appended claims the invention may be practiced otherwise than as specifically described.

What is claimed:

1. A method for simultaneously protecting and coloring a metal, said method being characterized by the steps of applying to a surface of the metal an aqueous dispersion of:

- (a) a water-soluble dichromate of a metal having a valence greater than one;
- (b) a compatible reducing agent for the dichromate;
- (c) a resin; and
- (d) a pigment,

the reducing agent being one that causes the chromium of the dichromate to be reduced to trivalent condition when the dispersion is heated to a temperature of at least about 280° F., the concentration of the reducing agent being such that from about 70 to 95% of the chromium is so reduced, and the pigment being in a concentration of about 10 to about 75% by weight of the dichromate, and heating the metal so coated to a temperature between about 280° F. and 450° F. to dry the applied dispersion and cause the above reduction, the quantity of dispersion applied to the metal being adjusted to give a coating weight after the heating of at least 100 milligrams per square foot.

2. The method of claim 1 in which the pigment is selected from the class consisting of phthalocyanine pigments, TiO<sub>2</sub>, carbon, and iron oxide.

3. The method of claim 1 in which the dispersed resin is in a concentration by weight not greater than twice the weight of the dichromate.

4. The method of claim 3 in which the dispersion is applied by spraying.

5. The method of claim 4 in which the spraying is carried out with a stream of compressed gas directed to evaporate off at least about three-fourths of the dispersant before the spray reaches the metal surfaces, and the coating weight after the heating is at least 1000 milligrams per square foot.

6. The method of claim 1 in which the metal is plain carbon steel and the dispersion contains metallic zinc particles less than 50 microns in size.

7. The method of claim 1 in which the dichromate is zinc dichromate.

8. The product produced by the process of claim 1.

9. The method of claim 1 in which the metal is plain carbon steel and the surface to which the dispersion is applied has a grain boundary etch.

10. The method of claim 1 in which the resin is an acrylic resin.

11. The method of claim 7 in which the drying and reduction of the coating is completed in not more than five seconds.

12. The method of claim 7 in which the resin is an acrylic resin and the drying and reduction is effected by momentarily bringing the coated metal to the heating temperature.

13. In the method of protecting metals against corrosion by applying an aqueous solution of a member se-

lected from the class consisting of chromic acid and dichromates of metals having a valence greater than 1, said solution also containing a reducing agent compatible with said member, the proportion of the reducing agent being such that the applied solution upon curing at a temperature of 250° F. is converted to a coating in which from 40 to 95% of the chromium is in trivalent form, the improvement by which said solution is applied to a casting of a metal of the class consisting of aluminum and zinc while said casting is at a temperature of approximately 500° F. to cause the coating to be promptly cured and partially decomposed.

14. In the method of protecting a metal against corrosion by applying to the surface of the metal an aqueous solution of chromic acid and a reducing agent compatible with the chromic acid at room temperature but which on drying and curing of the applied solution reduces 40 to 95% of the chromium of the chromic acid to trivalent condition, the improvement according to which the cured layer is made to present a pleasing color by substituting for the chromic acid the dichromate of a metal having a valence greater than one, dispersing in the aqueous solution a pigment in an amount from about 10 to about 75% by weight of the dichromate, and car-

rying out the curing at a temperature of at least 280° F. so that at least 70% of the chromium becomes reduced.

15. The product produced by the process of claim 14.

16. The combination of claim 14 in which the drying and curing of the coating solution is completed in not more than five seconds.

References Cited in the file of this patent

UNITED STATES PATENTS

|    |           |                 |       |                |
|----|-----------|-----------------|-------|----------------|
| 10 | 1,965,269 | Tostervd        | ----- | July 3, 1934   |
|    | 2,163,768 | Tanner          | ----- | June 27, 1939  |
|    | 2,206,064 | Thompson et al. | ----- | July 2, 1940   |
|    | 2,210,850 | Curtin          | ----- | Aug. 6, 1940   |
| 15 | 2,347,572 | Martin et al.   | ----- | Apr. 25, 1944  |
|    | 2,442,195 | Clenny          | ----- | May 25, 1948   |
|    | 2,562,117 | Osdal           | ----- | July 24, 1951  |
|    | 2,768,103 | Schuster et al. | ----- | Oct. 23, 1956  |
|    | 2,768,104 | Schuster et al. | ----- | Oct. 23, 1956  |
| 20 | 2,773,623 | Schuster et al. | ----- | Dec. 11, 1956  |
|    | 2,853,406 | Schuster et al. | ----- | Sept. 23, 1958 |
|    | 2,902,390 | Bell            | ----- | Sept. 1, 1959  |
|    | 2,911,332 | Schuster et al. | ----- | Nov. 3, 1959   |

UNITED STATES PATENT OFFICE  
CERTIFICATE OF CORRECTION

Patent No. 3,053,702

September 11, 1962

Ludwig K. Schuster et al.

It is hereby certified that error appears in the above numbered patent requiring correction and that the said Letters Patent should read as corrected below.

In the grant, line 4, and in the heading to the printed specification, lines 5 and 6, for "a corporation of Delaware", each occurrence, read -- a corporation of Pennsylvania --.

Signed and sealed this 16th day of April 1963.

(SEAL)

Attest:

ERNEST W. SWIDER  
Attesting Officer

DAVID L. LADD  
Commissioner of Patents